

Jan. 26, 1943.

D. T. HADDOCK

2,309,585

APPARATUS FOR MAKING TERNE SHEETS OR PLATES

Filed Feb. 12, 1941

FIG. 1.



FIG. 2.



FIG. 3.



FIG. 4.



Inventor:

DANIEL T. HADDOCK,  
by: *John E. Jackson*  
his Attorney.

## UNITED STATES PATENT OFFICE

2,309,585

## APPARATUS FOR MAKING TERNE SHEETS OR PLATES

Daniel T. Haddock, Tucson, Ariz.

Application February 12, 1941, Serial No. 378,644

4 Claims. (Cl. 91—12.7)

This invention relates to terne sheets or plates and, more particularly, to such apparatus as is employed therein.

Heretofore in making terne (lead-tin) sheets or plates, it was not possible to secure the desired amount of coating on the first pass of the sheet through the molten bath, which necessitated re-running the material several times therethrough until the desired weight of coating was attained. The weight of terne practically runs between 8 and 40 pounds, which figures express the weight of coating necessary to coat 112 sheets or plates, each 20" by 28" in size, or the equivalent thereof.

It is among the primary objects of this invention to deposit the exact amount of terne coating desired on a metallic sheet or plate by only one passage thereof through the molten bath.

To the accomplishment of these and other desirable objects and purposes, I have designed the present, preferred embodiments of the invention presented in the accompanying drawing forming a part of this specification and to which reference should be had in connection with the following detailed description, and in the drawing, for simplicity, like reference numerals have been employed to designate the same parts throughout the several views.

Figure 1 is a sectional view of a typical terne pot;

Figure 2 is an enlarged elevation of one of the rolls of the terne coating pot of Figure 1;

Figure 3 is an enlarged fragmentary area of the roll of Figure 2; and

Figure 4 is an enlarged cross-section of a portion of the roll of Figure 2 showing the depth and spacing of grooves on its outer surface which is used for 40 pound coatings.

Referring more particularly to the drawing, the numeral 2 designates a typical coating pot in which is retained molten terne (lead-tin) 3. As indicated by the arrows, the sheet to be coated is fed in any manner desired, through the flux box 4 at the entrance end of the pot and between guides 5 toward the exit end, during which it is coated on both sides with terne. The coated sheet is then fed through an oil box 6 and at the same time passes between a pair of driven rolls 8 which smooth the semi-molten coating, after which it emerges therefrom and is cooled by the atmosphere.

The present invention comprises material changes in the surface of either or both of these rolls 8. Heretofore, sheets coated with terne always ran light to weight of coating and if, as usual, a heavy coating was desired, they had to

be rerun through the pot one or more times in order to bring the thickness or weight of the coating up to the desired extent. Thus, in obtaining a 40 pound coating, as previously described, it was necessary to rerun a terne coated sheet at least twice through the molten bath.

In the art of coating with molten metals, most frequently the coating rolls are smooth. In terne coating it has been proposed to provide exit rolls corresponding to the rolls 8, described hereinbefore, which embody helical grooves, the helix of the groove of one roll opposing the helix of the groove of the opposing roll. At certain sustained speeds these rolls, embodying single helical grooves, function in such manner that there is deposited on the sheet or plate a terne coating of the desired weight. This constitutes an improvement over the smooth-faced rolls, the use of which necessitated rerunning. At somewhat increased speeds made necessary by change in consistency of the molten terne, the rolls having single helical grooves exert a wiping action which is deleterious to the obtaining of a coating of the required weight.

According to the teachings of the present invention, there is provided on the face of either or both of the rolls 8 opposed helical grooves which are identical in shape and pitch with the result that the surface of the said roll comprises even, diamond-shaped patterns and correspondingly even, separating grooves, the surfaces of the said patterns being substantially cylindrical.

It has been discovered that these opposed helical grooves on a single roll should be no deeper than 0.01", spaced approximately  $\frac{1}{8}$ " apart and substantially V-shaped, with the walls extending at substantially 60 degrees.

These opposed helical grooves may be formed by taking a spiral cut in one direction from one end of the roll to the other, reversing the direction of cut, and cutting identical grooves in the opposite direction, thereby producing on the surface of the roll a uniformly distributed matte of diamond-shaped projections as aforesaid. Thus, for example, for a roll of  $4\frac{1}{2}$ " diameter, each of the opposed helices would take a  $3\frac{1}{2}$ " lead.

The weight of coating obtained is more or less proportional to the size or the area of the opposed helical grooves, the larger the groove the greater the weight of coating and vice versa. In no case, however, should the groove exceed a depth of 0.01". It has been discovered that for obtaining a 20 pound terne coating, a depth of 0.004" is satisfactory. Accordingly, for various weights of coating it is only necessary to vary the

area of the diamond-shaped patterns, which is best accomplished by varying the depth of the grooves. It will be apparent, however, that the size of the area can also be changed by varying the space or pitch and shape of the groove.

When using rolls of approximately  $4\frac{1}{2}$ " with the opposed helical grooves given a  $3\frac{1}{2}$ " lead with  $\frac{1}{8}$ " between the bottoms thereof, and the grooves being substantially V-shaped with the sides thereof extending at substantially 60 degrees and of a depth of approximately 0.004", smooth and even 20 pound terne coatings may be obtained; and if the speed of the rolls is increased, necessitated by a change in the consistency of the molten terne, the coating will not vary therewith.

The  $3\frac{1}{2}$ " lead given the opposed helical groove in a roll of  $4\frac{1}{2}$ " diameter constitutes an angle of approximately 75 degrees, as shown in the developed surface of Figure 5 of the drawing. In a direction circumferentially of the roll the patterns are elongated, as distinguished from square. The increase in the angularity referred to hereinbefore from 75 degrees toward 90 degrees will result in further elongation in the direction stated, while a decrease in the angularity of 75 degrees will increase tendency toward a square. I have found, however, that the angle of 75 degrees, while susceptible of some variation in either direction, is ideal for the purpose stated.

While I have shown and described certain specific embodiments of the present invention, it will be understood that I do not wish to be limited exactly thereto, since various modifications may be made without departing from the scope of the invention as defined by the following claims.

This application is in part a continuation of an application Ser. No. 121,652 filed Jan. 21, 1937.

I claim:

1. In a machine for terne-coating sheets or plates, a pair of opposed rotary exit rolls, at least one of said rolls being only partially immersed in the oil bath of said machine and having opposed helical grooves, each of said opposed helical grooves being V-shaped and having a depth of no greater than 0.01", said grooves being substantially identical in shape and pitch to thereby provide even diamond-shaped patterns, the greatest dimensions of said diamond-shaped patterns being peripherally of the roll embodying the same, the surfaces of said diamond-shaped patterns being substantially cylindrical whereby heavy and even coatings may be secured in a single passage of the sheet or plate through the machine.

2. In a machine for terne-coating sheets or plates, a pair of opposed rotary exit rolls, at least one of said rolls being only partially immersed in the oil bath of said machine and having opposed helical grooves, each of said opposed helical grooves being V-shaped and having a depth of no greater than 0.01", said grooves being substantially identical in shape and pitch to thereby provide even diamond-shaped patterns, the greatest dimensions of said diamond-shaped patterns being peripherally of the roll embodying the same, the distance between the bottoms of parallel grooves being approximately  $\frac{1}{8}$ ", the surfaces of said diamond-shaped patterns being substantially cylindrical whereby heavy and even coatings may be secured in a single passage of the sheet or plate through the machine.

3. In a machine for terne-coating sheets or plates, a pair of opposed rotary exit rolls, at least one of said rolls being only partially immersed in the oil bath of said machine and having opposed helical grooves, each of said opposed helical grooves being V-shaped and having a depth of no greater than 0.01", said grooves being substantially identical in shape and pitch to thereby provide even diamond-shaped patterns, the greatest dimensions of said diamond-shaped patterns being peripherally of the roll embodying the same, the pitches of said grooves defining approximate 75° angles with respect to the roll axis, the surfaces of said diamond-shaped patterns being substantially cylindrical whereby heavy and even coatings may be secured in a single passage of the sheet or plate through the machine.

4. In a machine for terne-coating sheets or plates, a pair of opposed rotary exit rolls, at least one of said rolls being only partially immersed in the oil bath of said machine and having opposed helical grooves, each of said opposed helical grooves being V-shaped and having a depth of no greater than 0.01", said grooves being substantially identical in shape and pitch to thereby provide even diamond-shaped patterns, the greatest dimensions of said diamond-shaped patterns being peripherally of the roll embodying the same, the distance between the bottoms of parallel grooves being approximately  $\frac{1}{8}$ ", the pitches of said grooves defining approximate 75° angles with respect to the roll axis, the surfaces of said diamond-shaped patterns being substantially cylindrical whereby heavy and even coatings may be secured in a single passage of the sheet or plate through the machine.

DANIEL T. HADDOCK.